

1

3,751,367

## COMPOSITIONS COMPRISING BORON COMPOUNDS AND POLYPHENYL THIOETHERS

Frank S. Clark and Loren W. Bannister, St. Louis, Mo., assignors to Monsanto Company, St. Louis, Mo.  
No Drawing. Filed July 29, 1971, Ser. No. 167,463  
Int. Cl. C09k 3/00

U.S. Cl. 252—78

15 Claims

### ABSTRACT OF THE DISCLOSURE

Compositions comprising polyphenyl thioethers, polyphenyl ethers-thioethers or mixtures thereof and a triphenylboroxin exhibit improved corrosiveness toward copper and silver without loss of oxidative stability. Such compositions are useful as functional fluids.

This invention relates to compositions comprising polyphenyl thioethers, polyphenyl ethers-thioethers or mixtures thereof, containing from 3 to 8 aromatic groups and a corrosion inhibiting amount of a triphenylboroxin. The compositions of this invention are useful as functional fluids.

Polyphenyl thioethers and polyphenyl ether-thioether combinations have found wide application as functional fluids due to their excellent thermal stability and lubricity. For example they have been found to be valuable as hydraulic fluids and as lubricants in motor operation, particularly in jet engines, and as heat transfer agents. Two of the most rigorous demands on fluids are made by jet aircraft hydraulic systems and jet engine lubrication systems. For example, as the speed and altitude of operation of jet powered aircraft increases, lubrication problems also increase because of higher operating temperatures and higher bearing pressures resulting from the increased thrust needed to obtain higher speeds and altitudes. Thus, the service conditions encountered by functional fluids become increasingly severe, and therefore, the useful life of such fluids is shortened.

The useful life of any lubricant or hydraulic fluid can be adjudged on the basis of many criteria such as the extent of viscosity increase, the extent of corrosion to metal surfaces in contact with the lubricant and the extent of engine deposits. Those skilled in the art have found various ways to improve lubricants and to thus retard or prevent the effects which shorten the useful life of a lubricant. Thus, for example, small amounts of other materials, or additives, can be added to lubricants in order to affect one or more of the properties of the base lubricant. However, it is difficult, especially as operating temperatures are increased, to find additives which will still perform the function for which they are added and yet not inject other problems.

Therefore, an object of this invention is to extend the useful life of polyphenyl thioethers, polyphenyl ether-thioethers or mixtures thereof by reducing their corrosivity toward certain metals without adversely affecting oxidative stability of the ethers.

These and other objects will become evident upon consideration of the following specification and examples.

The above and other object of this invention are carried out by admixing polyphenyl thioethers, polyphenyl ether-thioethers or mixtures thereof with a corrosion inhibiting amount of a triphenylboroxin. The ether-boron compositions of this invention exhibit reduced corrosiveness toward metals without an adverse effect on oxidative stability of the base ether and thus have an extended service life even under the severe conditions encountered in jet engines and other devices operating at temperatures of the order of 600° F. The compositions exhibit markedly reduced corrosion toward copper and silver.

2

The improved compositions of this invention comprise a major amount of ether base fluid of the formula



wherein  $R^2$  is phenyl, alkyl-substituted phenyl wherein the alkyl is of not more than 4 carbon atoms, alkoxy-substituted phenyl wherein the alkoxy is of not more than 4 carbon atoms or halogenated phenyl wherein the halogen is bromine, fluorine or chlorine,  $R^3$  is phenylene, alkyl or alkoxy-substituted phenylene wherein the alkyl contains no more than 4 carbon atoms or halogenated phenylene wherein the halogen is fluorine, bromine or chlorine, and  $Y$  is selected from oxygen and sulfur but at least one of the  $Y$ 's is sulfur and  $a$  is an integer having a value of 1 to 6 and a corrosion inhibiting amount of at least one triphenylboroxin of the formula



wherein  $R$  is alkyl of not more than 4 carbon atoms, alkoxy of not more than 4 carbon atoms, halogen (Cl, Br and F) haloalkyl of not more than 4 carbon atoms and 3 halogen atoms (Cl, Br and F) haloalkoxy of not more than 4 carbon atoms and 3 halogen atoms (Cl, Br and F), phenoxy, phenylmercapto or  $NO_2$ ,  $R^1$  is halogen (Cl, Br and F) or alkyl of not more than 4 carbon atoms,  $n$  is an integer of 0 to 3 and  $m$  is an integer of 0 to 2.

Representative groups for  $R$  in the above formula include halogen (Cl, Br and F),  $NO_2$ , phenoxy, thiophenoxy, alkyl such as methyl, ethyl, propyl, isopropyl, n-butyl, sec-butyl and t-butyl, alkoxy such as methoxy, ethoxy, butoxy, haloalkyl such as chloromethyl, bromomethyl, chloroethyl, bromoethyl, trichloromethyl, tribromomethyl, trifluoroethyl, dichloroethyl, chloro-n-propyl, bromo-n-propyl, bromo-n-butyl, bromo-tert-butyl, 1,3,3-trichlorobutyl and 1,3,3-tribromobutyl and haloalkoxy such as chloromethoxy, 1,2-dichlorobutoxy and fluoropropoxy. Representative groups for  $R^1$  include the halogen and alkyl listed above for  $R$ .

Representative boron compounds of the above formula include

triphenylboroxin  
tri(3-methylphenyl)boroxin  
tri(4-n-butylphenyl)boroxin  
tri(2,4-dimethylphenyl)boroxin  
tri(4-methoxyphenyl)boroxin  
tri(4-chloromethylphenyl)boroxin  
tri(3-fluoromethylphenyl)boroxin  
tri(4-trifluoromethylphenyl)boroxin  
tri(4-chlorophenyl)boroxin  
tri(2,4-dichlorophenyl)boroxin  
tri(3-fluorophenyl)boroxin  
tri(4-phenoxyphenyl)boroxin  
tri(4-nitrophenyl)boroxin  
tri(4-phenylmercaptophenyl)boroxin  
tri(2-fluoro-4-methylphenyl)boroxin  
tri(2-methyl-4-chlorophenyl)boroxin  
tri(2-chloro-4-phenoxyphenyl)boroxin

The amount of triphenylboroxin employed in the compositions of this invention can range from about 0.01 to about 1.5% by weight. It is preferred to employ the acids in the compositions of this invention in amounts of from

about 0.05 to about 01.5% by weight based upon the total composition.

The polyphenyl thioethers employed in the composition of this invention have from 3 to 8 benzene rings and from 1 to 7 sulfur atoms with the sulfur atoms joining the benzene rings in chains as ether linkages.

The term "polyphenyl thioether" as used herein means a compound or physical mixture of compounds wherein all of the Y's in the above formula are sulfur. The term "polyphenylether-thioether" as used herein means compounds or physical mixtures of compounds wherein at least one but not all of the Y's in the above formula is sulfur.

The compositions of this invention contain a major amount of the polyphenyl thioether or polyphenyl ether-thioether base stock, i.e., at least 50% by weight of the total composition comprises an ether. It is preferred that at least 60% by weight of the composition be an ether base stock and even more preferred that at least 85% by weight of the total composition comprise an ether.

Illustrations of the alkyl-substituents present in the phenyl and phenylene groups of the ethers are for example, methyl, ethyl, propyl, butyl and the like. Illustrations of the alkoxy-substituents are, for example, methoxy, ethoxy, propoxy, butoxy and their isomers.

The compositions of this invention can also contain from 0.01 to 10% by weight of the total composition of a dialkyl hydrogen phosphite extreme pressure additive. The dialkyl hydrogen phosphites useful are those wherein the alkyl groups contain from 1 to 12 carbon atoms. The alkyl groups are for example, methyl, ethyl, propyl, isopropyl, butyl, sec-butyl, t-butyl, hexyl, decyl, isodecyl, dodecyl and the like.

Illustrative of the polyphenyl thioethers which can be employed as base stocks for the compositions of this invention are the bis(phenylmercapto)benzenes. For example

m-bis(phenylmercapto)benzene  
o-bis(phenylmercapto)benzene  
p-bis(phenylmercapto)benzene  
bis(m-phenylmercaptophenyl)sulfide  
bis(o-phenylmercaptophenyl)sulfide  
bis(p-phenylmercaptophenyl)sulfide  
(m-phenylmercaptophenyl)(o-phenylmercaptophenyl)sulfide  
p-phenylmercapto-m'-phenylmercapto diphenyl sulfide  
o-bis(o-phenylmercaptophenylmercapto)benzene  
p-bis(p-phenylmercaptophenylmercapto)benzene  
p-bis(o-phenylmercaptophenylmercapto)benzene  
p-bis(m-phenylmercaptophenylmercapto)benzene  
m-bis(p-phenylmercaptophenylmercapto)benzene  
o-bis(p-phenylmercaptophenylmercapto)benzene

and the like and mixtures thereof.

Illustrative of the mixed polyphenyl ether-thioether compounds which can be employed as base stocks in the compositions of this invention are for example,

o-phenylmercapto-m-phenoxy benzene  
p-phenylmercapto-o-phenoxy benzene  
m-phenoxy-p-phenylmercapto benzene  
o-phenylmercapto-p'-phenoxydiphenyl sulfide  
o-phenylmercapto-m'-phenoxydiphenyl sulfide  
o-phenoxy-m'-phenylmercaptodiphenyl sulfide  
m-phenoxy-p'-phenylmercaptodiphenyl sulfide  
o-phenoxy-p'-phenylmercaptodiphenyl sulfide  
p-phenoxy-p'-phenylmercaptodiphenyl sulfide  
o-phenoxy-o'-phenylmercaptodiphenyl sulfide  
o,o'-bis(phenylmercapto) diphenyl ether  
o-phenylmercapto-m-phenylmercaptodiphenyl ether  
o-phenylmercapto-p-phenylmercaptodiphenyl ether  
m-(m-phenylmercaptophenylmercapto) (m-phenoxyphenylmercapto)benzene  
[m-(m-phenylmercaptophenylmercapto)phenyl]  
[m-(m-phenoxyphenylmercapto)phenyl]sulfide

3-(m-phenylmercaptophenylmercapto)-3'-(m-mercaptophenoxy)diphenyl sulfide  
3,3'-bis(m-phenylmercaptophenylmercapto)diphenyl ether  
5 3-(m-phenylmercaptophenylmercapto)-3'-(m-phenoxyphenoxy)diphenyl sulfide  
4-(m-phenylmercaptophenylmercapto-4'-(m-phenylmercaptophenoxy)diphenyl ether  
3-(m-phenylmercaptophenylmercapto)-3'-(m-phenoxyphenylmercapto)diphenyl ether  
4,4'-bis(m-phenylmercaptophenoxy)diphenyl sulfide  
4,4'-bis(m-phenoxyphenylmercapto)diphenyl sulfide  
3-(m-phenoxyphenylmercapto)-3'-(m-phenylmercaptophenoxy)diphenyl sulfide  
15 3,3'-bis(m-phenylmercaptophenoxy)diphenyl ether  
4-(m-phenylmercaptophenylmercapto)-4'-(m-phenoxyphenoxy)diphenyl ether  
3-(p-phenylmercaptophenoxy)-3'-(p-phenoxyphenoxy)diphenyl sulfide  
20 3-(m-phenylmercaptophenoxy)-3'-(m-phenoxyphenylmercapto)diphenyl ether  
3,3'-bis(m-phenoxyphenylmercapto)diphenyl ether and  
3-(m-phenoxyphenylmercapto)-3'-(m-phenoxyphenoxy)diphenyl sulfide  
25 In addition to the foregoing compounds, the phenyl and phenylene of such compounds can contain substituents, such as alkyl of 1 to 4 carbon atoms, alkoxy of 1 to 4 carbon atoms and halogen such as chlorine, bromine and fluorine. Examples of such compounds are as follows:  
4,4'-bis(m-tolylmercapto)diphenyl ether  
3,3'-bis(m-tolylmercapto)diphenyl ether  
2,4'-bis(m-tolylmercapto)diphenyl ether  
3,4'-bis(m-tolylmercapto)diphenyl ether  
35 3,3'-bis(p-tolylmercapto)diphenyl ether  
3,3'-bis(xylylmercapto)diphenyl ether  
4,4'-bis(xylylmercapto)diphenyl ether  
3,4'-bis(xylylmercapto)diphenyl ether  
4,4'-bis(m-isopropylphenylmercapto)diphenyl ether  
40 3,3'-bis(m-isopropylphenylmercapto)diphenyl ether  
2,4'-bis(m-isopropylphenylmercapto)diphenyl ether  
3,4'-bis(p-tert-butylphenylmercapto)diphenyl ether  
4,4'-bis(p-tert-butylphenylmercapto)diphenyl ether  
3,3'-bis(p-tert-butylphenylmercapto)diphenyl ether  
45 3,3'-bis(2,4-di-tert-butylphenylmercapto)diphenyl ether  
3,3'-bis(3-chlorophenylmercapto)diphenyl ether  
4,4'-bis(3-chlorophenylmercapto)diphenyl ether  
3,3'-bis(m-trifluoromethylphenylmercapto)diphenyl ether  
4,4'-bis(m-trifluoromethylphenylmercapto)diphenyl ether  
50 3,4'-bis(m-trifluoromethylphenylmercapto)diphenyl ether  
2,3'-bis(m-trifluoromethylphenylmercapto)diphenyl ether  
3,3'-bis(p-trifluoromethylphenylmercapto)diphenyl ether  
3,3'-bis(o-trifluoromethylphenylmercapto)diphenyl ether  
3,3'-bis(m-methoxyphenylmercapto)diphenyl ether  
55 3,4'-bis(m-isopropoxyphenylmercapto)diphenyl ether  
3,4'-bis(m-perfluorobutylphenylmercapto)diphenyl ether  
2-(m-tolylxy)-2'-phenylmercaptodiphenyl sulfide  
2-(p-tolylxy)-3'-phenylmercaptodiphenyl sulfide  
2-(o-tolylxy)-4'-phenylmercaptodiphenyl sulfide  
60 3-(m-tolylxy)-3'-phenylmercaptodiphenyl sulfide  
3-(m-tolylxy)-4'-phenylmercaptodiphenyl sulfide  
4-(m-tolylxy)-4'-phenylmercaptodiphenyl sulfide  
3-xylyloxy-4'-phenylmercaptodiphenyl sulfide  
3-xylyloxy-3'-phenylmercaptodiphenyl sulfide  
65 3-phenoxy-3'-(m-tolylmercapto)diphenyl sulfide  
3-phenoxy-4'-(m-tolylmercapto)diphenyl sulfide  
2-phenoxy-3'-(p-tolylmercapto)diphenyl sulfide  
3-phenoxy-4'-(m-isopropylphenylmercapto)diphenyl sulfide  
70 3-phenoxy-3'-(m-isopropylphenylmercapto)diphenyl sulfide  
3-m-toloxo-3'-(m-isopropylphenylmercapto)diphenyl sulfide  
4-(m-trifluoromethylphenoxy)-4'-phenylmercaptodi-phenyl sulfide  
75

5

3-(m-trifluoromethylphenoxy)-4'-phenylmercaptodi-phenyl sulfide  
 2-(m-trifluoromethylphenoxy)-3'-phenylmercaptodi-phenyl sulfide  
 3-(m-trifluoromethylphenoxy)-3'-phenylmercaptodi-phenyl sulfide  
 3-(p-chlorophenoxy)-3'-phenylmercaptodiphenyl sulfide  
 3-(m-bromophenoxy)-3'-phenylmercaptodiphenyl sulfide  
 bis[m-(m-chlorophenoxy)phenyl]sulfide  
 m-bis[3-(p-methylphenylmercapto)phenoxy]benzene  
 m-bis[3-(m-trifluoromethylphenoxy)phenylmercapto]benzene  
 m-bis[3-(m-bromophenoxy)phenylmercapto]benzene  
 3,3'-bis[m-(p-methylphenylmercapto)phenoxy]diphenyl sulfide  
 3,4'-bis[m-(p-methylphenylmercapto)phenoxy]diphenyl sulfide  
 3-(p-xenoxy)-3'-phenylmercapto diphenyl sulfide,  
 and the like and mixtures thereof. It is also contemplated within the scope of this invention to employ mixtures of polyphenyl ether-thioethers as base stocks.

The triphenylboroxins useful in the compositions of this invention are well known to the art and can be prepared by dehydration of phenylboric acids as set forth in The Organic Chemistry of Boron, Academic Press, New York, 68 (1961). Phenylboric acids can be prepared by the procedures set forth in articles by R. M. Washburn et al., Advances in Chemistry Series, 32, 208 (1961) and W. Gerrard, The Organic Chemistry of Boron, Academic Press, New York, 59 (1961) or U.S. Pat. No. 3,092,652.

The following examples serve to further illustrate the invention. All parts are parts by weight unless otherwise expressly set forth.

## EXAMPLES

Polyphenyl thioether-polyphenyl ether-thioether lubricant compositions are prepared by combining 0.10 gm. of various triphenylboroxins with 100 grams of a thioether of the following composition:

|                                                    | Percent by wt. |
|----------------------------------------------------|----------------|
| Meta-bis(phenylmercapto)benzene                    | 50             |
| Bis(m-phenoxyphenyl)sulfide                        | 12.5           |
| (m-Phenoxyphenyl)(m - phenylmercaptophenyl)sulfide | 23.5           |
| Bis(m-phenylmercaptophenyl)sulfide                 | 12.65          |
| 3 ring and 5 ring thioethers                       | 1.35           |

and containing 10 parts per million of a dimethyl silicone antifoam agent (Dow-Corning-200, 350 cs. fluid). After stirring at 40° C. to dissolve the anhydride, the mixture is cooled to room temperature and filtered. Lubricant compositions without boron additives were used as control.

The useful life of a functional fluid can be determined on the basis of many criteria such as the extent of viscosity increase (oxidative stability) and corrosiveness toward metals under the conditions of use. The major bench scale method used for evaluating the oxidative stability of a functional fluid is the procedure given in Federal Test Specification 791, Method 5308 according to which the lubricant composition is heated at a specified temperature in the presence of certain metals and oxygen and the viscosity increase of the lubricant is determined.

The compositions of this example were tested according to the procedure of Federal Test Specification 791, Method 5308, i.e., 500° F. for 48 hours with five liters/hour of air in the presence of steel, copper, silver, titanium, magnesium alloy and aluminum alloy. Information with respect to corrosiveness of the compositions to metals was also obtained. However, only the results upon copper and silver are reported since all the compositions tested has essentially no effect on the other metals employed. Viscosity measurements were made according to ASTM Method D-445-53T using a Cannon-Fenske modified Ostwald viscosimeter. The control base fluid ether

6

and the compositions of this invention exhibited substantially the same viscosity increase. The corrosiveness to metals was determined by weighing metal specimens of known size before and after the test. Results and further details are given in the table below

TABLE

| Boron additive                           | Metal attack, mg./cm. <sup>2</sup> |      |
|------------------------------------------|------------------------------------|------|
|                                          | Cu                                 | Ag   |
| None (control).....                      | 2.4                                | 0.5  |
| Triphenylboroxin.....                    | 0.04                               | 0.10 |
| Tri(3-trifluoromethylphenyl)boroxin..... | 0.20                               | 0.07 |
| Tri(3-fluorophenyl)boroxin.....          | 0.23                               | 0.04 |

From the above it is clearly evident that the compositions of this invention exhibit markedly reduced corrosivity toward metals with no loss of oxidative stability and therefore have an extended useful life.

It will be appreciated that the compositions of the invention may also contain other additives, such as oxidation inhibitors, rust and corrosion inhibitors, antifoaming agents, detergents, viscosity index improvers such as polymeric materials for example, polyacrylate alkyl esters, polymethacrylate alkyl esters, polyoxyalkylene compounds, polyurethanes and the like. Such additives are usually employed in amounts as low as 10 parts per million for antifoaming agent to as much as 15 parts by weight of the total compositions for viscosity index improvers.

30 While the invention has been described with respect to specific examples and embodiments, it is to be understood that the invention is not limited thereto and that it can be variously practiced within the scope of the following claims.

The embodiments of this invention in which a particular property or privilege is claimed are defined as follows:

1. Composition consisting essentially of a major amount of a base fluid selected from the group consisting of polyphenyl thioethers, polyphenyl ether-thioethers, and mixtures thereof having the formula

wherein R<sup>2</sup> is phenyl, alkyl-substituted phenyl wherein the alkyl is of not more than 4 carbon atoms, alkoxy-substituted phenyl wherein the alkoxy is of not more than 4 carbon atoms or halogenated phenyl wherein the halogen is bromine, fluorine or chlorine, R<sup>3</sup> is phenylene, alkyl or alkoxy-substituted phenylene wherein the alkyl contains no more than 4 carbon atoms or halogenated phenylene wherein the halogen is fluorine, bromine or chlorine, and Y is selected from oxygen and sulfur but at least one of the Y's is sulfur and a is an integer having a value of 1 to 6 and a corrosion inhibiting amount of at least one triphenylboroxin of the formula



wherein R is alkyl of not more than 4 carbon atoms, alkoxy of not more than 4 carbon atoms, halogen selected from Cl, Br and F, haloalkyl of not more than 4 carbon atoms and 3 halogen atoms selected from Cl, 70 Br and F, haloalkoxy of not more than 4 carbon atoms and 3 halogen atoms selected from Cl, Br and F, phenoxy, phenylmercapto or  $\text{NO}_2$ ,  $R^1$  is halogen selected from Cl, Br and F or alkyl of not more than 4 carbon atoms, 75  $n$  is an integer of 0 to 3 and  $m$  is an integer of 0 to 2.

2. Composition of claim 1 wherein the boroxin is present in an amount from about 0.01% to about 1.5% by weight based on the total weight of the composition.

3. Composition of claim 1 wherein the boroxin is tri-phenylboroxin.

4. Composition of claim 1 wherein the boroxin is tri-(3-trifluoromethylphenyl)boroxin.

5. Composition of claim 1 wherein the boroxin is tri-(3-fluorophenyl)boroxin.

6. Composition of claim 1 wherein the boroxin is tri-(3-methylphenyl)boroxin. 10

7. Composition of claim 1 wherein the boroxin is tri-(4-methoxyphenyl)boroxin.

8. Composition of claim 1 wherein  $n$  is zero.

9. Composition of claim 1 wherein  $m$  is zero.

10. Composition of claim 1 wherein R is alkyl and 15  $m$  is zero.

11. Composition of claim 1 wherein R<sup>1</sup> is halogen and  $n$  is zero. fl

12. Composition of claim 1 wherein R is haloalkyl and 20  $m$  is zero.

13. Composition of claim 1 wherein R<sup>2</sup> is phenyl and R<sup>3</sup> is phenylene.

14. Composition of claim 1 wherein R is phenyl.

15. Composition of claim 1 wherein R is haloalkyl and R<sup>1</sup> is alkyl.

**References Cited**

**UNITED STATES PATENTS**

|   |           |         |                       |           |
|---|-----------|---------|-----------------------|-----------|
| 5 | 2,312,208 | 2/1943  | Clayton et al. -----  | 252—75    |
|   | 3,108,966 | 10/1963 | Dadura et al. -----   | 252—46.3  |
|   | 3,518,287 | 6/1970  | Rinse -----           | 252—389 X |
|   | 3,518,314 | 6/1970  | Giesecking -----      | 252—78 X  |
|   | 3,538,166 | 11/1970 | Campbell et al. ----- | 252—78 X  |
|   | 3,078,305 | 2/1963  | Dobratz -----         | 260—545   |
|   | 3,125,528 | 3/1964  | Kay et al. -----      | 252—49.6  |
|   | 3,321,529 | 5/1967  | Campbell -----        | 252—78 X  |
|   | 3,450,770 | 6/1969  | Campbell et al. ----- | 252—78 X  |
|   | 3,455,846 | 7/1969  | Bannister -----       | 252—78 X  |

**OTHER REFERENCES**

"Chemical Abstracts," vol. 59, 1679 (f) (1963).

LEON D. ROSDOL, Primary Examiner

H. A. PITLICK, Assistant Examiner

U.S. CL. X.R.

252—46.3, 49.6, 389 R; 260—545, 606.5 B